# EUROPEAN PATENT SPECIFICATION

(11) **EP 0 095 798 B1**
(45) Date of publication and mention of the grant of the patent: **08.04.1987**
(21) Application number: 83200677.9
(22) Date of filing: 11.05.1983
(51) Int. Cl.: C22F 1/00, C22C 9/04, C22C 9/08

(54) **Process for thermally treating heat recoverable metallic articles and articles thereby obtained**
Verfahren zur Wärmebehandlung von Gegenständen aus Formgedächtnislegierungen und Gegenstände nach diesem Verfahren hergestellt
Procédé pour le traitement thermique d'objets métalliques doués de propriétés de reprise thermique et produits obtenus selon ce procédé

(30) Priority: 13.05.1982 NL 8201986; 05.08.1982 NL 8203120
(43) Date of publication of application: 07.12.1983
(73) Proprietor: Leuven Research & Development V.Z.W., B-3000 Leuven (BE)
(72) Inventor: Delaey, Luc, B-3060 Bertem (BE); Van Humbeeck, Jan, B-3030 Heverlee (BE)
(74) Representative: Dopchie, Jean-Marc

## Description

The invention relates to heat recoverable metallic articles and to processes for producing them with the purpose of improving their heat recoverability as defined below, e.g. by maintaining said property stable in time.

Heat recoverable articles are known which consist of an alloy containing e.g. copper, zinc and aluminium as described e.g. in the US patent No. 3.783.037.

Heat recoverability is to be understood hereinafter as to comprise pseudo-elasticity, shape memory, reversible shape memory, good mechanical vibration damping and change in electrical conductivity which properties all relate to the transformation of an ordered Beta-crystal structure as metallic compound to a martensitic crystal structure. The temperatures which define the change of the crystal structure when following the transformation cycle are known as As, A_{f}, Mₛ and M_{f}.

It is known that the As-temperatures tend to change when the articles are maintained at a temperature in the martensitic state, which temperature is situated relatively close to this transformation temperature. However, varying As and Mₛ are very inconvenient in applications where a high reliability of the operation of a device is linked to the crossing of a temperature level which depends on these transformation temperatures of the heat recoverable article. For instance, a substantial change of As is not permissive in the operation of a fire safety device, an alarm device in a chemical process which is continuously exposed to a high temperature or for controlling a window opening in a greenhouse which is adjusted at an optimal temperature.

In some ranges of composition of copper-zinc- aluminium alloys, particularly with more than 5% of aluminium-e.g. with about 6%-and with 21% zinc-the As temperature can increase so much after a certain time of holding the article at room temperature that the transformation from martensite to the beta crystal structure (on further heating) can be traversed by a recrystallization reaction Cu-Zn-AI alloys and alloys similar thereto or related therewith are therefore not always usable as such with respect to their properties of heat recoverability.

In this application the alloy compositions useful for the invention will be given in weight percentages, wherein the sum of all metallic components are calculated as a 100% composition and wherein additions as some or other non-metallic phase such as oxides are not considered. For Cu-Zn-AI alloys, substituting elements of the metallic phase in the composition will be regarded as a substitution of copper because aluminium and zinc are the main elements which determine the characteristic transformation temperatures Mₛ, M_{f}, As and A_{f}.

The alloys, applicable according to the invention, have an As temperature which generally, but not necessarily, corresponds to the Mₛ temperature of which only differs by a few °C from it and which moreover is above 0°C and preferably even above room temperature. Below these temperatures, the diffusion rate of vacancies in the lattice is sufficiently low to reduce the change of As as is intended by the invention.

The process according to the invention is especially applicable in those circumstances where during the thermal treatment no equilibrium phase of alpha or gamma type nor a transition phase such as bainite is formed, which would lead to an equilibrium phase. In other words the thermal treatment will be executed in such a way that these equilibrium or transition phases are not formed. However the presence of aluminium-containing precipitates of intermetallic compounds, such as e.g. cobalt, which have a high grain boundary plane energy, seem to be able to favourably influence the stability of the heat recoverability over a longer time.

In a treatment which is described by Schofield and Miodownik (Metals Technology-April 1980 p. 167-173), it is the main purpose to stabilize at the same time As and Mₛ on keeping the alloy at a temperature above Mₛ which alloy was previously quenched to this temperature above Mₛ and without having been submitted to a deformation. When staying at this temperature (for an alloy Cu-Zn-AI with 4% Al) the ordering parameter S of the Beta-lattice changes. Hence all characteristic temperatures As, A_{f}, Mₛ and M_{f} change thereby together.

The present invention however, aims at keeping As at a substantially unchanged level, even after a long stay of the heat recoverable articles in martensitic condition at As or just below As. The stay in these conditions is generally and also hereafter called ripening. In practice a very slow heating has often the effect of ripening. The tendency however, to raise the temperature As by ripening does not exist for the Mₛ and M_{f}-temperatures. For alloys with a higher As, e.g. at 150°C, the effect of ripening is more difficult to master, but the invention can usefully be applied for ripening temperatures between e.g. 50°C and 120°C.

The invention consists in reducing the number of lattice vacancies in the beta structure by a factor of at least one hundred before its transformation to martensite and even to bring them to a negligible level (in the order of 10-⁷ to 10-⁹. With a concentration of vacancies which is too high, either a change in the parameter S of long range ordering in the martensitic stage is reached or a pinning of lattice vacancies with nuclei and with grain boundary planes in the martensite is reached. These martensite grain boundary plates are the boundaries of the different martensite plates or twin plates which form in the martensitic structure. The boundary plates are not grain boundaries as such, but the boundaries of areas (subgrains) which are in a fixed orientation relationship with respect to each other and in relation to the crystallographic parameters.

The invention will be further clarified with reference to the adjoined drawings in which
Figure 1 shows the influence of the different heat treatments on the transformation temperatures;
Figure 2 shows the composition range in the copper, zinc and aluminium diagram within which the invention is applicable;
Figure 3 is a scheme of a suitable cooling curve: temperature decrease (ordinate) as a function of time (abscissa);
Figure 4 shows an alternative cooling curve;
Figure 5 is a graph representing an example of the influence on As according to a second process according to the invention.

Figure 1 shows in a schematic way for an article made of an alloy containing 73.5% copper, 20.5% zinc and 6% aluminium how the hysteresis loop, which is a characteristic of heat recoverability, changes when running through the transformation cycle of the beta-crystal structure towards martensite as a function of temperature. The figure is relative to the extent that the different loops were drawn separate from each other to avoid confusion through overlaps. The characteristic of heat recoverability was measured as the change in electrical resistivity R (in ordinate) with temperature. Analogously also another parameter can be used. A type indication of the hysteresis loop 1 with the characteristic temperatures is shown in frame 2. A rod made of the alloy mentioned above is, after fabrication annealed for a first time at 750°C for 15 minutes and subsequently immediately quenched and kept for 20 minutes at 10°C above Ms(=60°C) prior to being further cooled in the air. The hysteresis loop recorded hereafter is shown by the line sections 3 and 4.

An identical rod which after this treatment was subjected to a 5% deformation in the martensite phase and heated again to above A, has a first thermal cycle according to the line sections 5 and 6. It can be noted that As has been shifted upwards as a consequence of the deformation in martensite. The following cycles again approach the line sections 6 and 4, in other words, As again drops to its former level (and also A_{f} decreases strongly).

An identical rod which is directly quenched to a temperature of 10°C above Mₛ and which is kept there for a long time (two hours) before being cooled down in the air to the martensitic state, then goes through a cycle according to the line sections 6 and 4. In case of 3% deformation in the martensitic state the loop deforms according to the line sections 7 and 4 to return to the line sections 6 and 4 after a few cycles.

If however, the process according to the invention is applied on a slightly modified composition, then an equilibrium cycle is obtained existing of the line sections 8 and 9 whereby the deformation of the martensitic phase broadens the hysteresis loop towards the line sections 9 and 10. After repeating the cycle a few times, the loop will again coincide with the line sections 8 and 9. This avoids a strong shifting of As.

Figure 2 shows as an example the composition range of the copper, zinc, aluminium diagram where the invention is very well applicable. The compositions lie between the points 11, 12, 13 and 14 shown in Table 1 and can be completed with the already discussed subsidiary elements such as for example cobalt. A limited amount of accidental subsidiary elements is thereby not excluded. The transformation temperature may then shift with the composition. The connecting line between the points 11 and 14 corresponds with an As transformation temperature of about 0°C and that between the points 13 and 12 with a transformation temperature As of about 190°C.

This diagram is based on the As temperatures and has been derived from "Metallwissenschaft und Technik", 31st year, issue No. 12, December 1977, pages 1326, where a similar diagram is based on the Mₛ temperatures. However, the analysis accuracy of these brass alloys is more problematic than the accuracy with which the transformation temperature can be measured. For the phenomena further described in this Application the temperature measurement is a determining factor after a standardized heat treatment. Indeed, the transformation temperature takes automatically account of the accidental presence of subsidiary elements or undesired precipitate formation.

The alloys to which the invention relates, include the ternary Cu-Zn-AI alloys which have an As temperature above 0°C and preferably above 20°C because at lower temperatures the diffusion speed becomes so small that a change of As due to ripening will be hardly noticable.

Table I shows by way of example target compositions (weight %) within which the invention can be applied:

As explained further on, these alloys possess at a temperature To a disordered beta-crystal structure in the absence of a precipitate of an equilibrium phase or of a transition phase, which may lead to an equilibrium phase and at a temperature below Mₛ, but higher than 0°C the alloy consists of martensite with a low concentration of lattice vacancies resulting from a reduction of concentration of lattice vacancies in the beta lattice structure by a factor of at least one hundred before their transformation. The alloy will optionally contain between 0.01 and 2% cobalt, between 0.01 % and 0.1 % boron, between 0% and 8% manganese and between 0% and 4% of nickel.

The invention relates also to a process for treating heat recoverable articles defined above with the temperatures As, A_{f}, Mₛ, M_{f} as features determining the recoverability.

According to this process the articles are cooled or quenched down from a disordered beta-crystal structure at elevated temperature To at least to a lower temperature T₁. These articles are kept for a sufficiently long time in the beta-crystal structure above the Mₛ temperature to stabilize the temperatures Mₛ, M_{f}, As, A_{f} at their equilibrium level, after which the articles are cooled down to the martensitic state below Mₛ. The term equilibrium level is meant herein to refer to the situation where the transformations always occur at the same respective temperatures upon repetitive application of the heating and cooling cycles, e.g. after deformation. According to the invention the concentration of lattice vacancies is reduced and an increase in As temperature after ripening is counteracted (whereas also the other transformation temperatures Mₛ and M_{f} are kept constant).

In a first process according to the invention the reduction of the number of lattice vacancies is obtained by quenching the material of the articles from the disordered higher temperature beta-crystal structure (at To) to a first temperature range T₁ in the beta structure, to keep the articles at these temperatures for a time interval t₁, to cool the material down to a second temperature range T₂, to maintain this temperature for a second time interval t₂, and subsequently to cool the articles down to the martensitic state below M_{f}.

The limits imposed on these time and temperature parameters are relative, i.e. the imposed treatment time may be shorter according as the temperature becomes higher.

In some cases the treatment times t₁ or t₂ may be so short that cooling in the air or in the furnace are sufficiently slow within a given time interval, to pass through the appropriate temperature ranges to obtain the desired stability of the As temperature. This also depends on the alloy composition. The temperature T₁ is for example 50°C higher than T₂ and lower than the alpha or gamma precipitation or the beta-recrystallization limits, and lies (depending on alloy and treatment time) preferably between 150°C and 500°C. The treatment time t₁ is preferably as short as possible, e.g. from a few seconds to 30 minutes, preferably between 10 seconds and'10 minutes. The temperature T₂ is higher than the Mₛ temperature and smaller than or equal to 0.7 T_{cDO3}, whereby T_{cDO3} is in absolute scale the critical temperature at which the D03 superlattice is formed from the B₂ superiattice. The treatment time t₂ must satisfy a minimum criterion and may extend from 1 minute to a few hours, preferably from 5 minutes to 2 hours. Since a great number of vacancies are absorbed in the grain boundaries, especially the treatment time t₁ may be strongly limited when an alloy with a fine grain structure is used, for example when the average grain size is inferior to 200 µm.

Figure 3a shows the temperature evolution in time for an article which is submitted to a stepwise heat treatment such as described above in the first process according to the invention. The point of departure is an annealing operation at high temperature in the beta-crystal structure which, for most alloys is conducted at 750°C (To) for a minimum duration of e.g. 5 minutes and preferably 15 minutes.

After quenching from To, the article is kept in point 15 of the graph at temperature T, for the time t, to be cooled further down towards T₂ for a time t₂, according to line 16, prior to cooling it further in a conventional way to below M_{f} according to the line 17.

A first test rod of a ternary alloy of 73.5% copper, 20.5% zinc and 6.0% aluminium was annealed at 750°C for 15 minutes, quenched in water at 80°C, kept for two hours at this temperature and then cooled until full transformation into martensite. When passed through a thermal cycle, a check rod showed an Mₛ of 60°C and an As of 62°C. The check rod was then divided into pieces and stored in a ripening test at different temperatures for different durations. At 25°C and after 7 days a ΔAₛ=3°C was measured. At 60°C and after 1 day the ΔAₛ=10°C, after 7 days it was 17°C.

A second test rod, which after having been cooled down was kept at 250°C for 5 minutes and subsequently further cooled as the first test rod, (hence after further quenching to 80°C and maintaining at this temperature for 2 hours and then cooling down to under M,), shows under comparable conditions in the ripening test a ΔAₛ which is less than half that of the first test rod. The evolution of the transformation temperatures was measured on the basis of the electrical resistivity to avoid parasitic effects of mechanical deformation.

In a second process according to the invention the article is kept at a temperature T₂ for a predetermined time as in the first process. Instead of carrying out a treatment at T₁, a content of 0.01% to 2% and preferably less than 1% and around 0.4% of copper can be substituted by a subsidiary element such as cobalt or by cobalt in combination with another metal. Then under suitable annealing conditions precipitates with high grain boundary plane energy are produced which have an average size smaller than 10 µm and preferably smaller than 5 µm. They are insoluble below the temperatures at which the equilibrium phases alpha and gamma are dissolved in the disordered beta-crystal structure. The element cobalt which forms a metallic compound together with aluminium may also be substituted by the elements palladium and platinum. These elements may even be partially, and for at most 50%, be replaced by titanium, chromium or nickel or by a combination thereof. This mixture of elements will be designated; hereinafter, as cobalt, insofar as they produce similar effects of grain refinement and uniformly distributed precipitates.

The boundaries of the grains and of the precipitate with high grain boundary plane energy probably absorb a great number of lattice vacancies. A similar effect is obtained in an alternative way by the addition of boron up to 0.1% preferably below 0.05% and in particular between 0.01 % and 0.03%. If, for example, owing to an extra annealing operation, these alloys have an average grain size of more than 200 µm, then a treatment time t, is preferred at T₁.

With the second process according to the invention it is also possible to quench an alloy, with eg. a precipitate of an aluminium-cobalt compound and with an average grain size of less than 200 µm, directly down to the temperature T₂ as shown by the dotted line 18.

In a third process according to the invention a heat recoverable article as used in the first process is quenched from the high-temperature disordered beta-crystal structure (at To) to a temperature T₃ below T₁ and above Mₛ where the metallic lattice is in the beta superlattice, but quenching may take place in a medium which has a temperature in the area of T₂. The treatment time t₃ at this temperature is set at a minimum for obtaining a uniform temperature T₃ throughout the article after which the temperature is preferably returned to T₁ as quickly as possible and the treatment, as described in the first process, is applied: the article is again quenched to T₂ where it is held for a period t₂ prior to being further cooled down to the martensitic state.

Figure 3b shows the temperature evolution of a thermal treatment corresponding with the third process according to the invention. After an annealing treatment at 750°C (To) for 15 minutes, the treated article is quenched to a temperature T₃ above the Mₛ temperature and significantly below Tᵢ. This is shown by the line section 19 of the cooling curve 20. The temperature T₃ is selected between the uppermost limit shown by the dotted line 25 and the bottom limit 26.

The corresponding time t₃ is preferably limited to the minimum level to obtain a uniform temperature in the article. The main purpose of the preliminary cooling is to obtain a greater treatment efficiency for thicker objects. The reduction in lattice vacancies is mainly obtained through a combination of the subsequent treatment at temperature T, for a time t₁ and at T₂ for a time t₂.

In a fourth process according to the invention the heat recoverable article, similar to that in the third process, is initially quenched from To to a lower temperature, this time at a temperature at which transformation to martensite takes place, preferably even below M_{f}. Heating to a temperature at least equal to T₁ must then follow immediately. This quenching treatment is applicable to some alloys, for example to an alloy containing 70% copper, 24% zinc and 4% aluminium. As for other alloys, for example composed of 73% copper, 21% zinc and 6% aluminium, the possibility of using shape memory characteristics is strongly reduced except in combination with certain production methods, such as hot drawing or extrusion. In some cases, an additional annealing treatment in the beta-crystal structure is necessary. In other cases, the shape memory is recoverable by rapid heating and holding at a temperature above T₁ for a very short time.

Figure 4 shows the cooling curve 21 of an article corresponding with the fourth process according to the invention. The quenching treatment from To is conducted at a temperature below M_{f}, after which it is heated to a temperature T₁ in a beta-crystal structure for a time t,, followed by a second treatment time t₂ after cooling to a lower temperature T₂ also in the beta-crystal structure. The further cooling to below M_{f} may be conducted without special precautionary measures.

As an alternative, a slowed-down cooling as from T₁ according to the dotted line 22 can be applied, for example in a furnace; so that the treatment time in the T₂ temperature range is equivalent to the proposed time t₂.

This fourth method has been advantageously applied after extrusion or hot rolling alloys into elongated articles such as wire and profiles. The heat deformation provides a high concentration of lattice defects. It is assumed that through the intermediate treatments at T₁ and T₂ more lattice vacancies can be absorbed in dislocation clusters and in the grain boundaries with the consequence that hence the concentration of lattice vacancies in martensite is considerably reduced.

Although quenching below the M_{f} temperature is appropriate, a quenching temperature between Mₛ and M, is also applicable. The quenching treatment is applied until above Mₛ for those alloys whereby the heat recoverability of the article would be jeopardized or endangered.

The treatment temperatures T₁ and T₂ and the treatment times t₁ and t₂ are preferably optimized on the basis of a limited test on a collection of samples.

The third and fourth process according to the invention also have practical significance to alloys of which the time required to form a precipitate from an equilibrium phase such as alpha, gamma or bainite is very short. In a lower-temperature cooling medium, the tip of the T.T.T. curve can be more easily avoided because the cooling speed is higher. Afterwards the treatment time t, can be increased without danger of precipitation at T₁.

In the description of the different processes according to the invention no mechanical deformation of the article was mentioned neither in a beta-crystal structure nor at lower temperature or in martensite. Cold deformation produces a rise in As temperature, which disappears again after a number of thermal and deformation cycles. After these treatment cycles which may for example be carried out some 20 times, a reversible shape memory effect is produced. The article behaves as an undeformed material. The heat recoverability capacity can easily be quantified by measuring for example the electrical resistivity.

With the different processes according to the invention the overall average vacancy density in the martensite or beta-crystal structure is reduced by preferential absorption of vacancies in some places such as the grain boundaries.

Furthermore, the structure may contain a precipitate with high grain boundary plane energy such as an aluminium-cobalt compound, so that the average grain size is smaller than 200 µm. This kind of precipitate formation may also occur in the presence of boron. Alternatively or in addition thereto, an increased dislocation density may be achieved through hot deformation in the disordered beta-crystal structure.

The following test run in Table II is useful for 'determining the parameters for an individual alloy with the composition range according to Figure 2.

The transformation temperature As of all samples is then immediately determined by means of resistivity measurements. All samples are returned to the martensitic state all for the same duration, e.g. two days at the same temperature, e.g. 2°C-3°C below the determined As. The As temperature is measured again. In this manner the different AS can be determined. Circumstances causing disturbing precipitation or other inconveniences are avoided.

The treatment parameters (such as e.g. treatment temperatures and stress) at temperatures T₁ and T₂ during the cooling process are therefore dependent upon the Mₛ temperature, the composition of the alloy out of which the article is composed and the absolute temperature at which for this composition the vacancies are reduced to a lower level.

For a cooling profile corresponding with the second process according to the invention, the influence of the ripening on As is shown in Figure 5. Articles made of an alloy of 73.5% copper, 20.5% zinc and 6% aluminium are compared with articles of an alloy of 73.1% copper, 20.5% zinc and 6% aluminium, 0.39% cobalt and 0.024% titanium. Owing to the influence of the annealing conditions on the transformation temperatures in the presence of e.g. cobalt, either in combination with titanium or not, the annealing took place each time at 750°C for 15 minutes after which quenching took place down to 80°C (T2) for 20 minutes (t₂). In case of further cooling to martensite, an As temperature of circa 60°C was found in both cases on the basis of measurements of the electrical resistivity. Subsequently successive measurements of As were conducted after various ripening times in the martensitic state at 60°C. The line 23 shows a value of ΔAₛ without the addition of cobalt-titanium. The line 24 shows the influence of ΔAₛ for articles of an alloy containing additions of cobalt and titanium after the thermal treatment produced a grain size of less than 200 µm.

In another example an alloy comprising 73.5% Cu, 20.5% Zn and 6% AI (M=₆₀°C) (in the form of a plate strip with a thickness of 1 mm) was betatized for 15 minutes at 750°C and quenched into water at 80°C. It was maintained at 80°C for two hours and then cooled in the air to room temperature. The sample was heated again to 55°C (=As) for some time and the ΔAₛ was determined:

Similar strip samples with same composition, shape and dimensions as above, were betatized at the same conditions and subsequently quenched down into hot oil at 250°C and held there for five minutes whereafter they were further quenched down to 80°C, and maintained there for two hours. Upon further cooling down in the air to room temperature and reheating for a certain time to 55°C resp. 45°C, the following ΔAₛ-values were found:

The heat treatment according to the invention results thus in a substantial decrease in ΔAₛ.

The invention is not limited to the Cu-Zn-AI containing alloys mentioned hereinbefore. It is also applicable e.g. to alloys which contain (apart from unavoidable impurities) 4-40% zinc, 1-12% aluminium, 0-8% manganese, 0―4% nickel, 0,005-1 % boron and the balance copper. The zinc content is then preferably 5-32% and the aluminium content 3-10%.

In practice the heat treatments on the shape memory alloys according to the invention enable them be used as actuator for temperature control. A change in temperature can thus be identified and signalized by the articles of the invention between a lower temperature which is lower than or equal to Aₛ of the alloy and a higher temperature which is (preferably) at least equal to A_{f} of the alloy. The change in shape or tendency to such change which occurs at this change in temperature then forms the signal which permits identification of the change in temperature. The difference between the higher and the lower temperature can thereby be smaller than 50°C and the lower temperature can be at room temperature or above.

According to the invention it is now possible to store the thermo-responsive actuator for a longer time at the lower temperature without creating a substantial upward shift in the As temperature. Apparatuses or devices comprising said actuators are of course within the contemplation of the invention. These actuators then comprise heat treated articles described above as means which enable them to reproducibly change in shape or a to tend to such change upon crossing a predetermined temperature range with the actuator.

## Claims

1. A heat recoverable article comprising an alloy which at a temperature To possesses a disordered beta-crystal structure and at a temperature T₁ lower than To an ordered beta-crystal structure in the absence of a precipitate of an equilibrium phase or of a transition phase, which may lead to an equilibrium phase and that at a temperature below Mₛ, but higher than 0°C the alloy consists of martensite with a low concentration of lattice vacancies resulting from a reduction of the concentration of lattice vacancies in the beta lattice structure by a factor of at least one hundred before its transformation to martensite, the article having a composition by weight percent in the ternary copper-zinc- aluminium diagram within the limit points (11) 64% Cu, 35% Zn, 1 % Al; (12) 74% Cu, 21 % Zn, 5% Al; (13) 87.5% Cu, 0% Zn, 12.5% Al; (14) 86% Cu, 0% Zn, 14% AI and optionally contains between 0.01% and 2% cobalt, between 0.01% and 0.1% boron, between 0% to 8% manganese and between 0% and 4% of nickel.

2. An article according to claim 1, characterized in that the cobalt content is less than to 1%.

3. An article according to claim 1, characterized in that the alloy contains less than 0.05% boron.

4. An article according to any of claims 1 to 3, characterized in that the alloy has an average grain size smaller than 200 pm.

5. A heat recoverable article comprising an alloy which at a temperature To possesses a disordered beta-crystal structure and at a temperature T, lower than To an ordered beta-crystal structure in the absence of a precipitate of an equilibrium phase or of a transition phase, which may lead to an equilibrium phase and that at a temperature below Mₛ, but higher than 0°C the alloy consists of martensite with a low concentration of lattice vacancies resulting from a reduction of the concentration of lattice vacancies in the beta lattice structure by a factor of at least one hundred before its transformation to martensite, the article having a composition of 4 to 40% zinc, 1 to 12% aluminium, 0 to 8% manganese, 0 to 4% nickel 0.005 to 1 % boron and the balance copper.

6. An article according to claim 5, characterized in that it comprises 5-32% zinc and 3-10% aluminium.

7. A process of producing a heat recoverable metallic article according to any of claims 1 to 5 with temperatures As, A,, Mₛ, M_{f} as characteristics of recoverability, comprising the steps of quenching the article from a temperature level To at which the article has a beta-crystal structure to a first temperature range (Tᵢ), which is lower than the recrystallisation limit, holding it there during a first time interval (t₁) which is smaller than 30 minutes, immediately thereafter cooling down the article to a second temperature range (T₂) which is between the Mₛ temperature and 0.7 T_{cDO3}, wherein T_{cDO3} in absolute scale is the critical transition temperature of a D03 superlattice towards the B2 superlattice for a second time interval (t₂) of at least one minute and thereafter cooling down the article below M_{f} to its martensitic state.

8. A process according to claim 7, characterized in that the first temperature range T₁ is lower than 500°C.

9. A process according to claim 7, characterized in that the first time interval t₁ is between ten seconds and ten minutes.

10. A process according to claim 7, characterized in that the second time interval t₂ is at least five minutes to 2 hours.

11. A process according to claim 7, characterized in that the articles in disordered beta-crystal structure at the temperature To are submitted to an annealing treatment for at least five minutes.

12. A process according to claim 7, characterized in that the articles in disordered beta-crystal structure at the temperature To are thermally deformed.

13. A process according to claim 12, characterized in that the thermal deformation comprises in an extrusion treatment.

14. A process according to claim 7, characterized in that the metal articles are quenched from a disordered beta-crystal structure at a temperature To to the level of the temperature range T₃ below T₁ and above the Mₛ-temperature and where the metallic lattice is in the beta superlattice and are held in this temperature range for a limited time interval (t₃) limited to the minimum level to obtain a uniform temperature level in the article, after which they are heated again to the first temperature range T₁ and again quenched to the second temperature range T₂ where they are held for a period of time (t₂) prior to being further cooled down to the martensitic state.

15. A process according to claim 7, characterized in that the metal articles are quenched from the disordered beta-crystal structure at a temperature To to below the Mₛ temperature and are maintained at this temperature for a limited period of time after which they are again heated to the first temperature range T₁, and successively after having been held at this temperature for a time interval (t,), again quenched to this second temperature range T₂ where they are held for a period of time (t₂) and subsequently cooled down to full transformation to a martensitic state.

16. Thermoresponsive actuator comprising means for identifying and signalizing a change in temperature which means include heat recoverable articles according to any of the claims 1 to 6, characterized in that they are able to reproducibly change in shape or to tend to such change by crossing a temperature range from below the Aₛ of the article, which is at room temperature or above, and up to above its A_{f}.

## Patentansprüche

1. Durch Wärme in den alten Zustand rückkehrfähiger Gegenstand, umfassend eine Legierung, die bei einer Temperatur Tₒ eine ungeordnete Beta-Kristallstruktur und bei einer Temperatur Tᵢ, niedriger als Tₒ, eine geordnete Beta-Kristallstruktur in der Abwesenheit eines Niederschlags einer Gleichgewichtsphase oder einer Übergangsphase besitzt, die zu einer Gleichgewichtsphase führen kann, und daß die Legierung bei einer Temperatur unterhalb von Mₛ, aber höher als 0°C, aus Martensit mit einer niedrigen Konzentration von Gitterfehlstellen besteht, die aus einer Herabsetzung der Konzentration von Gitterfehlstellen in der Beta-Gitterstruktur um einen Faktor von zumindest einhundert von ihrer Umwandlung in Martensit herrührt, wobei der Gegenstand eine Zusammensetzung in Gewichtprozent im ternären Kupfer-Zink-Aluminium-Diagramm innerhalb der Grenzpunkte (11) 64% Cu, 35% Zn, 1% AI; (12) 74% Cu, 21% Zn, 5% Al; (13) 87,5% Cu, 0% Zn, 12,5% Al; (14) 86% Cu, 0% Zn, 14% AI besitzt und fakultativ zwischen 0,01 % und 2% Kobalt, zwischen 0,01% und 0,1% Bor, zwischen 0% bis 8% Mangan und zwischen 0% und 4% Nickel enthält.

2. Gegenstand nach Anspruch 1, dadurch gekennzeichnet, daß der Kobaltgehalt weniger als bis 1% ist.

3. Gegenstand nach Anspruch 1, dadurch gekennzeichnet, daß die Legierung weniger als 0,05% Bor enthält.

4. Gegenstand nach einem beliebigen der Ansprüche 1 bis 3, dadurch gekennzeichnet, daß die Legierung eine mittlere Korngröße kleiner als 200 µm besitzt.

5. Durch Wärme in den alten Zustand rückkehrfähiger Gegenstand, umfassend eine Legierung, die bei einer Temperatur Tₒ eine ungeordnete Beta-Kristallstruktur und bei einer Temperatur T₁, niedriger als Tₒ, eine geordnete Beta-Kristallstruktur in den Abwesenheit eines Niederschlags einer Gleichgewichtsphase oder einer Übergangsphase besitzt, die zu einer Gleichgewichtsphase führen kann, und daß die Legierung bei einer Temperatur unterhalb von M_{S}, aber höher als 0°C aus Martensit mit einer niedrigen Konzentration von Gitterfehlstellen besteht, die von einer Herabsetzung der Konzentration von Gitterfehlstellen in der Beta-Gitterstruktur um einen Faktor von zumindest einhundert vor ihrer Umwandlung in Martensit herrührt, wobei der Gegenstand eine Zusammensetzung von 4 bis 40% Zink, 1 bis 12% Aluminium, 0 bis 8% Mangan, 0 bis 4% Nickel, 0,005 bis 1% Bor und das Gleichgewichtskupfer besitzt.

6. Gegenstand nach Anspruch 5, dadurch gekennzeichnet, daß er 5-32% Zink und 3-10% Aluminium umfaßt.

7. Verfahren zur Herstellung eines durch Wärme in den alten Zustand rückkehrfähigen metallischen Gegenstands nach einem beliebigen der Ansprüche 1 bis 5 mit Temperaturen Aₛ, A_{f}, Mₛ, M_{f} als Merkmalen für die Rückkehrfähigkeit in den alten Zustand, umfassend die Schritte, daß der Gegenstand aus einem Temperaturpegel Tₒ, bei dem der Gegenstand eine Beta-Kristallstruktur besitzt, auf einen ersten Temperaturbereich (T₁) abgeschreckt wird, der niedriger als die Rekristallisationsgrenze ist, er dort während eines ersten Zeitintervalls (t₁), das kleiner als 30 Minuten ist, gehalten wird, der Gegenstand anschließend sofort auf einen zweiten Temperaturbereich (T₂) abgekühlt wird, der zwischen der Mₛ-Temperatur und 0,7 T_{cDO3} liegt, wobei T_{cDO3} in der absoluten Skala die kritische Übergangstemperatur eines D03-Übergitters zum B2-Übergitter ist, für ein zweites Zeitintervall (t₂) von zumindest einer Minute, und der Gegenstand anschließend unter M_{f} zu seinem martensitischen Zustand abgekühlt wird.

8. Verfahren nach Anspruch 7, dadurch gekennzeichnet, daß der erste Temperaturbereich T₁ niedriger als 500°C ist.

9. Verfahren nach Anspruch 7, dadurch gekennzeichnet, daß das erste Zeitintervall t₁ zwischen zehn Sekunden und zehn Minuten ist.

10. Verfahren nach Anspruch 7, dadurch gekennzeichnet, daß das zweite Zeitintervall t₂ zumindest fünf Minuten bis 2 Stunden ist.

11. Verfahren nach Anspruch 7, dadurch gekennzeichnet, daß die Gegenstände in ungeordneter Beta-Kristallstruktur bei der Temperatur Tₒ für zumindest fünf Minuten einer Vergütungsbehandlung unterzogen werden.

12. Verfahren nach Anspruch 7, dadurch gekennzeichnet, daß die Gegenstände in ungeordneter Beta-Kristallstruktur bei der Temperatur Tₒ wärmeverformt werden.

13. Verfahren nach Anspruch 12, dadurch gekennzeichnet, daß die Wärmeverformung eine Strangpreßbehandlung umfaßt.

14. Verfahren nach Anspruch 7, dadurch gekennzeichnet, daß die Metallgegenstände aus einer ungeordneten Beta-Kristallstruktur bei einer Temperatur Tₒ zu dem Pegel des Temperaturbereichs T₃ unterhalb von T₁ und oberhalb der Mₛ-Temperatur abgeschreckt werden und wo das metallische Gitter im Beta-Übergitter ist, und in diesem Temperaturbereich für ein begrenztes Zeitintervall (t₃) gehalten werden, das auf den Minimalpegel begrenzt ist, um einen einheitlichen Temperaturpegel im Gegenstand zu erhalten, wonach sie wieder zum ersten Temperaturbereich T₁ erwärmt werden und wieder auf den zweiten Temperaturbereich T₂ abgeschreckt werden, wo sie für eine Zeitperiode (t₂) gehalten werden, bevor sie weiter zum martensitischen Zustand abgekühlt werden.

15. Verfahren nach Anspruch 7, dadurch gekennzeichnet, daß die Metallgegenstände aus der ungeordneten Beta-Kristallstruktur bei einer Temperatur Tₒ auf unter die Mₛ-Temperatur abgeschreckt werden und bei dieser Temperatur für eine begrenzte Zeitperiode gehalten werden, nach der sie wieder auf den ersten Temperaturbereich T₁ erwärmt werden, und nacheinander, nachdem sie bei dieser Temperatur für ein Zeitintervall (t₁) gehalten worden sind, wieder auf diesen zweiten Temperaturbereich T₂ abgeschreckt werden, wo sie während einer Zeitperiode (t₂) gehalten werden und nachher zur vollen Umwandlung zum martensitischen Zustand abgekühlt werden.

16. Auf Wärme ansprechender Schalter, umfassend Einrichtungen zur Identifizierung und Signalisierung eine Temperaturänderung, wobei die Einrichtungen durch Wärme in den alten Zustand rückkehrfähige Gegenstände gemäß einem beliebigen der Ansprüche 1 bis 6 enthalten, dadurch gekennzeichnet, daß sie in der Lage sind, sich in der Form reproduzierbar zu ändern, oder zu einer solchen Änderung durch Kreuzen eines Temperaturbereichs von unterhalb der Aₛ des Gegenstandes, die bei Zimmertemperatur oder darüber liegt, und bis zu oberhalb ihrer A_{f} zu führen.

## Revendications

1. Article métallique à récupérabilité thermique, comprenant un alliage, qui à une température Tₒ possède une structure cristalline B désordonnée et à une température T₁ inférieure à Tₒ une structure cristalline β ordonnée en l'absence d'un précipité d'une phase en équilibre ou d'une phase de transition, qui peut conduire à une phase en équilibre et qui, à une température inférieure à Mₛ mais supérieure à 0°C consiste en Martensite avec une faible concentration de vides réticulaires, résultant d'une réduction de la concentration des vides réticulaires dans la structure réticulaire β par un facteur d'au moins un centième avant sa transformation en martensite, l'article ayant une composition exprimée en pourcentage en poids dans un diagramme ternaire cuivre-zinc- aluminium aux points limites (11) 64% Cu, 35% Zn, 1% AI, (12), 74% Cu, 21% Zn, 5% AI; (13) 87,5% Cu, 0% Zn, 12,5% AI; (14) 86% Cu, 0% Zn, 14% AI, et pouvant contenir optionellement entre 0,01 % et 2% Cobalt, entre 0,01 % et 0,1 % de Bore, entre 0% et 8% de Manganèse et entre 0% et 4% de Nickel.

2. Article suivant la revendication 1, caractérisé en ce que la teneur en Cobalt est inférieure à 1 %.

3. Article suivant la revendication 2, caractérisé en ce que l'alliage contient moins de 0,05% de Bore.

4. Article suivant l'une de revendications 1 à 3, caractérisé en ce que l'alliage possède une dimension moyenne de grain inférieure à 200 µm.

5. Article métallique à récupérabilité thermique. comprenant un alliage, qui à une température Tₒ, possède une structure cristalline désordonnée et à une température T,, inférieure à Tₒ une structure cristalline β ordonnée en l'absence d'un précipité d'une phase en équilibre ou d'une phase de transition, pouvant conduire à une phase en équilibre et qui, à une température inférieure à Mₛ mais supérieure à 0°C, consiste en Martensite avec une faible concentration en vides réticulaires résultant d'une réduction de la concentration des vides réticulaires dans la structure réticulaire β par un facteur d'au moins un centième avant sa transformation en Martensite, l'article ayant une composition de 4 à 40% de Zinc, 1 à 12% d'Aluminium, 0 à 8% de Manganèse, de 0 à 4% Nickel, de 0,005 à 1 % de Bore, la balance étant de cuivre.

6. Article suivant la revendication 5, caractérisé en ce qu'il contient 5 à 32% de Zinc et 3 à 10% d'Aluminium.

7. Procédé de production d'articles métalliques à récupérabilité thermique, suivant l'une des revendications 1 à 5, avec des températures Aₛ, A_{f}, Mₛ, M_{f} comme caractéristiques de la récupérabilité, comprenant les étapes de trempage de l'article d'un niveau de température Tₒ, où l'article possède une structure cristalline β, à une première zone de température (T₁) inférieure à la limite de cristallisation,―de maintien à cette température durant un premier intervalle de temps (t₁), inférieur à 30 minutes, suivi immédiatement d'un refroidissement à une seconde zone de température (T₂) qui se trouve entre la température Mₛ et 0,7 T_{cDO3}, où T_{cDO3} à l'échelle absolue est la température critique de transition d'un super réseau D03 vers le super réseau B2-durant un second intervalle de temps (t₂) d'au moins une minute―l'article étant alors refroidi en dessous de M_{f} vers son état martensitique.

8. Procédé suivant la revendication 7, caractérisé en ce que la première zone de température T₁ est inférieure à 500°C.

9. Procédé suivant la revendication 7, caractérisé en ce que le premier intervalle de temps t, se trouve entre dix secondes et dix minutes.

10. Procédé suivant la revendication 7, caractérisé en ce que le second intervalle de temps t₂ est d'au moins de cinq minutes à 2 heures.

11. Procédé suivant la revendication 7, caractérisé en ce que les articles dans leur structure cristalline β désordonnée soient soumis à traitement de recuit d'au moins cinq minutes.

12. Procédé suivant le revendication 7, caractérisé en ce que les articles dans leur structure cristalline β désordonnée, subissent une déformation thermique à la température Tₒ.

13. Procédé suivant la revendication 12, caractérisé en ce que la déformation thermique comprend un traitement d'extrusion.

14. Procédé suivant la revendication 7, caractérisé en ce que les articles métalliques, à partir d'une structure cristalline β désordonnée à une température Tₒ, sont trempés à une zone de température T₃, inférieure à T₁ et supérieure à la température Mₛ, et où le réseau métallique est dans le super-réseau β, et sont maintenus dans cette zone de température pendant un intervalle de temps limité (t₃); réduit au minimum nécessaire pour obtenir un niveau de température uniforme dans l'articie,―pour être ensuite réchauffés à la première zone de température T₁ et retrempés dans la seconde zone de température T₂ où ils sont maintenus pendant une période de temps (t₂) avant d'être refroidis ultérieurement à l'état martensitique.

15. Procédé suivant la revendication 7, caractérisé en ce que les articles métalliques à partir d'une structure cristalline β désordonnée à une température To, sont trempés à une température inférieure à Mₛ et y sont maintenus durant un intervalle de temps limité pour être ensuite réchauffés à une température à la première zone de température T₁, y étant maintenus, à cette température, durant un intervalle de temps (tₗ), pour être ensuite, retrempés à la seconde zone de température T2 y étant maintenus, à cette température, durant un intervalle de temps (t₂) et refroidis par la suite pour la transformation totale à l'état martensitique.

16. Dispositif thermosensible de commande, comprenant des moyens pour identifier et signaler un changement de température, ces moyens comprenant des articles métalliques à récupérabilité thermique, suivant les revendications 1 à 6, caractérisé en ce qu'ils sont susceptibles, de manière reproductive, de changer de forme ou de tendre à changer de forme en traversant une zone de température, allant d'une température inférieure à la température de l'article, température de la chambre ou supérieure à celle-ci, jusqu'au dessus de sa température A_{f}.
